

Dec. 16, 1969

W. A. TAEBEL ET AL

3,484,278

PYROLYTIC BERYLLIA

Filed Oct. 7, 1965



FIG. 1



FIG. 2

INVENTORS:  
Wilbert A. Taebel &  
Gerard W. Hoekstra

by *Green and Durr*  
ATTORNEYS.

1

3,484,278

## PYROLYTIC BERYLLIA

Wilbert A. Taebel, 12 Beverly Drive, Towaco, N.J. 07082, and Gerard W. Hoekstra, 49 Seton Hall Drive, Oakland, N.J. 07436

Filed Oct. 7, 1965, Ser. No. 493,836

Int. Cl. C23c 13/02, 13/04

U.S. Cl. 117—106

1 Claim

### ABSTRACT OF THE DISCLOSURE

According to the invention BeO is deposited by vaporizing the basic formate of beryllium, heating the vapors to a temperature above their decomposition temperature in a region containing a surface heated to 250–600° C. whereupon dense BeO is deposited on the surface.

This invention relates to a process of preparing beryllia by the pyrolytic process and to the pyrolytic beryllia so produced.

Among the objects of the invention is to provide a process of preparing hard, dense and thick beryllia deposits.

Among other objects of the invention is to provide a relatively low temperature process for depositing hard, dense beryllia on a substrate.

Among still other objects of the invention is to provide an improved process for the production of pyrolytic beryllia.

Processes for depositing metal oxides by chemical vapor pyrolysis processes are known and may be classed generally into one of the following categories.

(1) Deposition by steam hydrolysis of certain metal halides.

(2) Deposition by oxidation of a metal halide with oxygen.

(3) Deposition by thermal degradation of a volatile metal compound containing chemically bonded oxygen.

The recommended deposition temperatures for the above reactions are quite high. Thus, Powell et al. in Vapor Plating, John Wiley & Sons (New York 1955), recommend temperatures of the order of 1000° C. for preparing oxide coatings by the steam hydrolysis of the halides. Again, Schlossberger et al. in WADC Technical Report 59-363, "Research on Pyrolytic Deposition of Thin Films," recommend a temperature for the preparation of oxide films by thermal degradation of compounds containing oxygen (such as ethyl silicate), of 1200° C. Others dealing with these processes have generally noted that temperatures of approximately 1000° C. or above are required for the preparation of even thin films.

This invention is based on the discovery that thick, dense, hard, deposits of beryllia can be obtained by the pyrolysis of an organic adduct of beryllium at a relatively low temperature of 300–600° C.

The deposits can be obtained of any desired thickness. The quality of the deposit is improved over deposits obtained at 1000° C., for example, because the total stress developed during deposition is less at the lower temperatures.

An "organic adduct of beryllium" may be defined as a compound in which the beryllium ion and the organic radical are held together by means of metal to oxygen to carbon bond, thus differing from organo-metallic compounds in which a metal to carbon bond exists. A satisfactory organic adduct is the basic formate,  $Be_4O(HCO_2)_6$ .

A process for making the basic organic adducts of beryllium (glucinium) with formic and other fatty acids is disclosed in Comptes Rendu Vo. 134,772 (1902).

2

The process of the invention is particularly useful for providing BeO film coatings for the oxidation protection of metals, particularly the refractive metals such as tungsten and molybdenum and for the oxidation protection of certain non-metals such as plastics, carbon (graphite), etc. The process is also useful for the production of lightweight impervious structures having a core of foamed or porous material and a coating of the dense pyrolytic BeO. Continuous refractory filaments may be prepared with a core of boron or nickel and a coating of BeO by this process.

The process also has applications in the production of complex shapes by selectively depositing the BeO over unmasked portions of a masked substrate.

Thus, the substrate on which the deposit is formed can be any material capable of withstanding temperatures of about 250° or more and can be of any shape. Coherent deposits are formed on a substrate of beryllia or other ceramic oxide as well as on the surfaces of refractory metals, plastics, etc.

In the process, the basic formate of beryllia is volatilized (sublimated) and is brought into contact with a preheated substrate in a closed chamber at sub-atmospheric, atmospheric or superatmospheric pressure. The substrate to be coated is heated to about 250–600° C. or even more if desired. One or both of the substrate and the vapor should be heated to the decomposition temperature of the vapor at the surface where the BeO is to be deposited which is between about 300–600° depending somewhat on the pressure. Lower rates of deposition are obtained at the lower temperatures.

In the drawing:

FIG. 1 shows an apparatus suitable for the deposition of beryllia by the process of the invention.

FIG. 2 is a photomicrograph (133×) of a cross-section of a deposit of beryllia on a ceramic beryllia substrate made according to the process.

The apparatus of FIG. 1 shows a bell jar 10 fitted on a suitable base 11 which is provided with a suitable pipe connection 12 for exhausting the bell jar 10. A ceramic pedestal 13 is provided to hold a beryllia plate 14 which in turn is provided with a heater means 15 connected to the outside through leads 16. A vaporizing chamber 17 for the organic adduct of beryllium is positioned on the heater 15 and beryllia plate 14. The vaporizing chamber 17 is provided with openings permitting the vapor to escape into the chamber means 20 which is adapted to surround a substrate to-be-coated 21. Heating means 22 for the substrate having leads 23 through the base 11 are provided. Thermocouples 24 and 25 to the vaporizing chamber 17 and deposition chamber respectively are provided.

The following example is given in detail to further illustrate how this invention may be carried out in practice. It is to be understood that the specific details given in the examples are not to be considered as limiting the scope of the invention.

### EXAMPLE 1

The apparatus as shown in FIG. 1 is employed with the basic formate of beryllium added to vessel 17 and with a slab of ceramically sintered beryllia as the substrate 21. The basic formate compound sublimes at 185° C. but in this case the bell jar is exhausted to a pressure of 30–35 mm. of Hg whereupon the basic formate begins to sublime at about 150° C. The BeO substrate 21 is heated to about 400° C. by heater 22. After about 10 minutes during which the basic formate compound is heated to 200° C., a deposit of BeO approximately 2–5 mm. in thickness is retained on the substrate. The deposit is similar to that shown in FIG. 2, the white portion being

the deposit and the lower darker portion being the original substrate. It will be noted that there is a substantially complete absence of pores in the deposited BeO whereas the sintered substrate shows its porous structure.

Beryllia can be deposited on metal or other surfaces in the same way. When the substrate is graphite or other form of carbon it is preferred to initiate the process in an inert atmosphere.

We claim:

1. The process of forming dense beryllia layers comprising:

providing the basic formate of beryllium,  
heating the basic formate of beryllium to form vapors  
of the same,

heating said vapors to a temperature above the decomposition temperature thereof in the region adjacent a surface heated to 250-600° C. whereby to deposit beryllia on said surface.

#### References Cited

Powell et al., Vapor Deposition, 1966, pp. 402 and 403  
relied upon.

ALFRED L. LEAVITT, Primary Examiner

A. GOLIAN, Assistant Examiner